

Jan. 12, 1943.

G. B. HOGABOOM

2,307,928

PROCESS AND APPARATUS FOR CLEANING METAL

Filed Feb. 24, 1939

2 Sheets-Sheet 1



Jan. 12, 1943.

G. B. HOGABOOM

2,307,928

PROCESS AND APPARATUS FOR CLEANING METAL

Filed Feb. 24, 1939

2 Sheets-Sheet 2

FIG. 2.



FIG. 4.



GEORGE B. HOGABOOM,  
INVENTOR

BY *Kingsbury*

ATTORNEYS.

## UNITED STATES PATENT OFFICE

2,307,928

PROCESS AND APPARATUS FOR CLEANING  
METALGeorge B. Hogboom, New Britain, Conn., assignor  
or to Hanson-Van Winkle-Munning Company,  
Matawan, N. J., a corporation of New Jersey

Application February 24, 1939, Serial No. 258,155

5 Claims. (Cl. 204—141)

In the usual process of electrolytic cleaning of metal, the metal is passed through, or hung in, a tank containing an alkaline solution and is cathodically connected in an electric circuit supplied with current at 6 to 12 volts. This produces a current density of at least 10 amp./sq. ft. and causes a vigorous evolution of hydrogen gas on the cathode. The improvement in the cleansing action over straight cleaning is believed to be due to several causes, including the formation of free alkali at the cathode, the mechanical action of the hydrogen bubbles on the surface of the cathode tending to lift the oil film and to assist in its emulsification, and the agitation of the solution, caused by the evolution of gas, which constantly brings fresh solution to the cathode surface.

A primary object of my invention is to render the electrolytic cleaning process more rapid and efficient by supplementing the effects of the usual process by a vigorous mechanical action brought about by throwing a forceful stream of cleaning solution against the metal. The cleaning action is accelerated by the impact of the solution, which physically tears away the dirt as it is loosened by the dissolving and electrolytic action. At the same time the dissolving action becomes more rapid, due to the continuous supply of new solution to the metal surface and its greater pressure against the metal surface.

A number of difficulties are encountered in electrolytic cleaning tanks as now operated. In the first place the cleaning is carried out in a tank which is constantly accumulating the dirt from the metal, leading to the danger of re-contamination of the metal from the scum in the tank.

In the second place, there is a gradual rise in the polarization voltage at the anodes, which is only partially corrected by making the anodes in the form of grids of very large surface.

In the third place, the temperature of the cleaning solution cannot be properly controlled. This temperature should be somewhat below the boiling point for best results, preferably about 180° F. The current generates heat, leading to boiling of the solution, which cannot be controlled, because the large anodes choking the tank do not permit effective use of cooling coils.

These and other difficulties are overcome by my invention. The cleaning operation is carried out in a cleaning chamber, to which cleaning solution is supplied from a reservoir and from which it constantly flows out, carrying with it the dirt removed from the metal. This removes the danger of the clean metal being soiled by an accumulation of dirty scum. The violent agitation of the solution in the cleaning chamber keeps the anode surfaces clean and prevents a continuous rise in the polarization voltage.

The temperature can be controlled because the reservoir is free to hold a cooling coil and the heat generated by the electric current is immediately carried off to the reservoir by the solution discharging from the cleaning chamber, the used solution being replaced by solution from the reservoir at the controlled temperature.

The invention is well suited to the cleaning of metal strip, the cleaning chamber, in this case, being arranged so that the strip will enter and leave it through gates and will be subjected in it to streams of cleaning solution. The cleaning solution can be allowed to escape from the cleaning chamber through the same gates by which the metal strip enters and leaves.

In electrolytic cleaning the cathodic cleaning is sometimes followed by anodic treatment of much shorter duration, for instance, where a deposit upon the metal from the cleaning solution in the cathodic treatment must be removed before electroplating. In accordance with my invention a cleaning chamber for cathodic treatment can be supplemented by a cleaning chamber for anodic treatment, and, in the case of continuous strip, the duration of treatment can be governed by the relative lengths of the cathodic and anodic cleaning chambers. Any number of cleaning chambers can be used and they can be arranged with cathodic and anodic chambers in alternation or in any other desired sequence.

Because of the greater efficiency of the cleaning process according to my invention, the apparatus required for the same work can be smaller. Where it is a question of treating strip which is running at a certain speed determined by other units of a combination of apparatus, the length of space required for the electrolytic cleaning can be considerably shortened.

While I have mentioned particularly the use of an alkaline cleaning bath, the invention is also applicable to electrolytic pickling and bright dipping.

The invention will be explained in detail by reference to two illustrative forms of apparatus shown in the accompanying drawings, wherein

Fig. 1 is a longitudinal vertical section of an electrolytic cleaning apparatus in accordance with my invention;

Fig. 2 is a vertical cross section of the same apparatus on the line 2—2 of Fig. 1;

Fig. 3 is a detail section on the line 3—3 of Fig. 1; and

Fig. 4 is a vertical longitudinal section of another form of apparatus in accordance with my invention.

In the apparatus shown in Figs. 1 to 3 a tank 1 is provided as a reservoir for alkaline cleaning solution 3, which may be of any of the well-known formulas. Above the tank are arranged

a series of cleaning chambers 5, 7, 9 and 11, etc., those shown being only a part of the full complement, though fewer may be employed if desired. As indicated by the break in the apparatus illustrated in Fig. 1, it may be considerably longer and the number of cleaning chambers correspondingly greater. This apparatus is designed for cleaning continuous strip metal indicated at 13. Each cleaning chamber is composed of two box-shaped members 15 and 17 provided with horizontal flanges 19, 21, 23, 25, 27, 29, 31 and 33. The flanges 27 and 29 and the flanges 31 and 33 are separated by sheets of insulating material 35, since in this particular apparatus the upper half of the cleaning chamber is to be electrically charged oppositely to the lower half. The two halves are clamped together by bolts 37 having metal washers 39 bearing upon washers 41 of insulating material, which protect the bolts 37 from contact with the flanges 29 and 33. At the upper end the bolts have nuts 43 bearing upon bridge clamps 45, and lock nuts 47.

The space 49 between flanges 19 and 21 constitutes an entrance gate through which the metal moves into the cleaning chamber and the space 51 between flanges 23 and 25 constitutes an exit gate from which the metal leaves the cleaning chamber. Within these spaces are buttons or ribs 53 of insulating material, to hold the metal strip 13 out of contact with the metal parts of the cleaning chamber. The bottom half of the cleaning chamber is fixed by screws 55 to channel bars 57 extending across the tank. The channel bars are supported by insulating posts 59 upon flanges 61 secured to the side walls of the tank 1. Screws 63 fix the channel bars to the insulating posts 59 and screws 65 secure the insulating posts to the flanges 61.

Within each half of each cleaning chamber is a pipe 67 provided with a longitudinal slot or series of perforations at 69 to emit a stream of cleaning solution directed against the upper and lower sides of the metal strip 13. The cleaning solution is supplied through pipes 71 connected by nipples 73 and sections of hose 75 to the pipes 67, and by a pipe 77 to the pressure side of a pump 79. The suction side of the pump is connected by a pipe 81 to the inside of the tank 1. A filter press 83 may be inserted in the pipe 77 to remove solids from the cleaning solution. Within the tank 1 is a cooling coil 85 supplied with coolant from a refrigerator unit 87.

Running along the series of cleaning chambers are bus bars 89 and 91 connected respectively to the positive and negative poles of a generator 93. The positive bus bar 89 is connected by a lead 95 to the upper half 15 of the first cooling chamber, while the negative bus bar 91 is connected by a lead 97 to the lower half 17 of the first cleaning chamber. The connections are reversed at the second cleaning chamber, where the upper half 15 is connected by a lead 99 to the negative bus bar 91 and the lower half 17 is connected by a lead 101 to the positive bus bar 89. The connections are thus alternated through the series of cleaning chambers.

Pairs of rollers 103, 105, 107, 109, 111 and 113 feed or support the metal strip 13 through the series of cleaning chambers. The pair of rollers 111 has the additional function of stripping the cleaning solution from the metal strip before it passes beyond the end wall of the tank 1.

The apparatus operates in the following manner:

The metal strip 13 is continuously fed through the cleaning chambers by the pairs of rollers 103, 105, 107, 109, 111, 113. Cleaning solution is pumped by pump 79 from the reservoir 1 through the filter press 83 to the pipes 67, where it jets out through the slots 69 in streams directed against the upper and lower surfaces of the strip 13. Electric current passes from the generator through the positive bus bar to the upper half 15 of the first cleaning chamber, thence through the cleaning solution to the lower half 17 of the cleaning chamber, from which it returns through lead 97 and bus bar 91 to the generator. At the second cleaning chamber the current from the positive bus bar 89 goes to the lower half 17 of the cleaning chamber, thence upward through the solution, the metal strip, and the solution again to the upper half 15 of the cleaning chamber, from which it returns through lead 99 to the negative bus bar 91. Thus in the successive cleaning chambers the current flows alternately downward and upward, and both surfaces of the metal strip receive cathodic treatment and anodic treatment. The current is concentrated principally across the spaces between flanges 19 and 21 and flanges 23 and 25, but some of the current also passes through other parts of the cleaning chamber. In the course of its travel through the cleaning chamber the metal strip 13 is subjected to the streams of cleaning solution issuing from the pipes 67 and the cleaning action due to solution and electrolytic activity is thus accelerated by the mechanical action of the streams of cleaning solution. The cleaning solution flows out of the cleaning chambers through the gates 49 and 51 from which it falls into the reservoir 1. This solution therefore constantly carries out of the cleaning chambers the dirt and grease removed from the metal. The insulating strips 35 extend into the cleaning chambers close to the edges of the metal strip 13 to guide the strip and to prevent short-circuiting of the electric current around the strip. There is considerable heat evolved in the cleaning chambers, much of which is carried to the reservoir with the returning cleaning solution and is absorbed by the refrigerating coils 85. The escape of cleaning solution from the cleaning chambers is controlled by the spacing of the flanges 19 and 21 and the flanges 23 and 25, as well as by the shape and size of the insulating buttons or ribs 53.

In the form of apparatus shown in Figs. 1-3 the metal receives the same periods of anodic and cathodic treatment, since in one cleaning chamber the upper side of the metal strip is being treated cathodically while the lower side is being subjected to anodic treatment and in the next cleaning chamber the conditions are reversed. It is sometimes desirable to make the duration of one kind of treatment longer than the other, particularly to give a longer cathodic treatment than anodic treatment. The apparatus shown in Fig. 4 is designed for this purpose. A reservoir 125 has mounted on it a cathodic cleaning chamber 127 and an anodic cleaning chamber 129, the manner of mounting the cleaning chambers on the reservoir being the same as before. In this case both the upper and lower halves of the cleaning chamber 127 are connected by leads 131 to the positive bus bar 89, while both halves of the anodic cleaning

chamber 129 are connected by leads 133 to the negative bus bar 91. Thus the current travels from the positive bus bar through the leads 131 and the upper and lower walls of cleaning chamber 127 through the cleaning solution to the strip 13, and longitudinally through the strip into cleaning chamber 129, where it passes through the cleaning solution to the upper and lower walls of the cleaning chamber 129 and through leads 133 to the negative bus bar 91. The portion of the metal strip 13 in the cleaning chamber 127 is therefore a cathode, while the portion in cleaning chamber 129 is an anode. The chamber 127 in this case is, for example, five times as long as the chamber 129, thus giving a cathodic treatment of, for instance, ten seconds and an anodic treatment of two seconds. In order to compensate for the greater electrode surface in chamber 127 than in chamber 129 there may be provided a shunt connection 135 with a rheostat 137. This shunt connection makes contact with the strip 13 by a brush 139 and is connected at its other end to lead 133. Conforming to the greater length of chamber 127 there are provided five jet pipes 67 above and five below the strip 13. If desired, the single long cathodic cleaning chamber 127 could be replaced by a number of short cleaning chambers giving a total length equal to the one long one.

Aside from the differences noted the second form of apparatus is the same as the first, having the same means for circulating the cleaning solution. These have not been shown in the drawings.

For electrolytic pickling and bright dipping an apparatus similar to that shown in Fig. 4 may be used, but with separate tanks under the two cleaning chambers. The pickling and bright dipping may be carried out as described in the patent to Hogaboom and King No. 1,865,470. The two chambers should be so proportioned that the metal can be given a treatment of 60 to 90 seconds in the first chamber and from 4 to 12 seconds in the second chamber. The circuit should be arranged as shown in Fig. 4, so that the metal will be cathodic in the first chamber and anodic in the second. The acid bath for the first chamber is preferably a sulphuric acid solution of 32° Bé. and is maintained at a temperature of 140° F. In the second chamber a 46° Bé. solution of sulphuric acid and a temperature not higher than 60° F. are preferred. The concentrations and temperatures may, however, be varied within the boundaries described in the aforesaid Patent No. 1,865,470. A current of 10 to 150 amperes per square foot of cathode surface may be used in the first chamber, and in the second chamber a current of 25 to 200 amperes per square foot of anode surface, depending upon the temperature of the solution.

While the term "cleaning solution" generally denotes an alkaline detergent bath, in the following claims it is to be construed in the broader sense of any electrolytic solution having a capacity for cleaning metal under the influence of an electric current.

I claim:

1. Apparatus for cleaning the surfaces of metal strip, comprising a cleaning chamber provided with entrance and exit gates for the strip to travel through longitudinally, said gates being

5 bounded by opposed electroconductive surfaces of large area provided with means for insulating the strip therefrom, means for applying cleaning solution to both sides of the strip in the cleaning chamber in opposed forceful transverse streams and thereby flushing the cleaning solution over the strip and out through said gates, and means for establishing an electric circuit passing through the surface of the strip and the cleaning solution in contact therewith.

10 2. Apparatus for cleaning the surface of metal strip, comprising means forming a cleaning chamber completely enclosed except for two gates for entrance and exit of the strip by longitudinal movement, means for applying cleaning solution to both sides of the strip in the cleaning chamber in opposed forceful transverse streams, whereby to flush cleaning solution over the strip in said chamber and out through said gates, and means for establishing an electric circuit passing through the surface of the strip and the solution in contact therewith.

15 3. In apparatus for cleaning continuous metal strip, a cleaning chamber comprising closely spaced electroconductive surfaces of large area provided with insulating means for spacing and guiding the strip between said surfaces, means for forcing opposed streams of cleaning solution against the opposite sides of the strip and through the spaces between said electroconductive surfaces and the two sides of the strip, and means for establishing an electric circuit passing through the surface of the continuous strip and the cleaning solution in contact therewith.

20 4. A method of electro-cleaning metal strip which comprises passing the strip longitudinally through the interior of an approximately closed cleaning chamber by way of restricted entrance and exit gates extending longitudinally of the strip, supplying cleaning solution to the interior of said cleaning chamber in opposed forceful transverse streams directed against the opposite faces of said strip within the interior of said cleaning chamber and thereby expelling a stream 25 of cleaning solution from the cleaning chamber along each face of the strip by way of at least one of said restricted gates through which said strip is longitudinally passing, and passing electric current between each face of the strip and the cleaning solution in contact therewith.

30 5. Apparatus for electro-cleaning metal strip which comprises an approximately closed housing forming an interior cleaning chamber of relatively large volume with relatively restricted entrance and exit gates for the metal strip in passing through said chamber, means for continuously feeding the metal strip through said cleaning chamber and gates, means for delivering cleaning solution into said interior cleaning chamber in the form of opposed forceful streams against the opposite faces of the metal strip passing therethrough, means for spacing the metal strip from the walls of said entrance and exit gates to provide passageways along the two faces of said strip for the escape of cleaning solution from the interior cleaning chamber outwardly through said gates, and means for passing electric current between the cleaning solution and strip.

GEORGE B. HOGABOOM.